

# United States Patent Office

2,983,610

Patented May 9, 1961

1

2,983,610

## SENSITIZATION OF PHOTOGRAPHIC EMULSIONS

Charles F. H. Allen, Wesley G. Lowe, and John Sagal, Jr., Rochester, N.Y., assignors to Eastman Kodak Company, Rochester, N.Y., a corporation of New Jersey

No Drawing. Filed Oct. 23, 1957, Ser. No. 691,811

4 Claims. (Cl. 96—108)

This invention relates to photographic silver halide emulsions, and more particularly, to a means for chemically sensitizing such photographic silver halide emulsions.

A number of methods have been previously proposed for increasing the sensitivity of photographic silver halide emulsions, other than methods of optical or spectral sensitization which involve the incorporation of certain dyes in the emulsions. The incorporation of dyes in the emulsions increases the optical range of sensitivity, whereas the incorporation of other materials known as chemical sensitizers increases the speed and generally the gamma of the emulsion without materially affecting the optical range of sensitivity. Many of the prior methods of enhancing sensitivity, other than the methods of spectral sensitization, leave much to be desired because the increase of sensitivity may be quite small or the increase in sensitivity is accompanied by excessive fog and/or excessively poor keeping qualities of the sensitized emulsions.

We have now found a method of increasing the sensitivity of photographic silver halide emulsions wherein the speed increases are quite substantial, while the fog and keeping qualities are not excessively affected, considering the magnitude of the increases in speed and gamma or contrast obtained.

It is, therefore, an object of our invention to provide photographic silver halide emulsions which have been chemically sensitized. Another object is to provide a method of preparing such sensitized emulsions. Still another object of our invention is to provide photographic silver halide emulsions which have increased sensitivity, without concomitant increases in fog, or poor keeping qualities, to a degree which might seriously affect the usefulness of the sensitized emulsions. Other objects will become apparent from a consideration of the following description and examples.

According to our invention, we have found that the sensitivity of an ordinary photographic silver halide emulsion can be materially increased by incorporating a formamidine sulfenic acid therein. Unsubstituted formamidine sulfenic acid is sometimes known as thiourea dioxide or imino-amino-methane sulfenic acid, depending upon the particular tautomeric form in which the compound is written. Formamidine sulfenic acid (or thiourea dioxide or imino-amino-methane sulfenic acid) can be represented as existing in the following state of equilibrium:



The formamidine sulfenic acids used in our invention

2

can be employed in the form of the free acid or in the form of their water-soluble salts (e.g. sodium, potassium, etc.). Formamidine sulfenic acids or salts which are particularly useful in practicing our invention can be represented by the following general formula:



10 wherein M represents a hydrogen atom or a solubilizing group or cation, such as sodium, potassium, etc., R, R<sub>1</sub> and R<sub>2</sub> each represents a hydrogen atom, a lower alkyl group (e.g., methyl, ethyl, n-propyl, n-butyl, etc., especially an alkyl group containing from 1 to 4 carbon atoms), an aryl group (e.g. phenyl, chlorophenyl, etc., especially a mononuclear aryl group of the benzene series), a heterocyclic radical (e.g., benzothiazolyl, piperidyl, etc.), etc.

15 The formamidine sulfenic acids useful in practicing our invention, or water-soluble salts of these acids, can be prepared in a known manner, such as the method referred to in Weber et al., U.S. Patent 2,339,309, issued January 18, 1944.

20 It has been previously proposed to incorporate various sulfenic acids in photographic silver halide emulsions for the purpose of increasing the stability thereof. For example, U.S. Patent 2,057,764 suggests the addition of alkane sulfenic acids, such as methane sulfenic acid, ethane sulfenic acid, etc., to photographic silver halide emulsions for the purpose of stabilization. However, as noted in this patent, these sulfenic acids have no detectable effect upon the sensitivity characteristics of the photographic silver halide emulsions. Contrasted with this behavior, the formamidine sulfenic acids of our invention have a profound effect upon the sensitivity characteristics of the photographic silver halide emulsions.

25 The preparation of silver halide emulsions involves three separate operations: (1) the emulsification and digestion of silver halide, (2) the freeing of the emulsion of excess soluble salts usually by washing, (3) the second digestion or after-ripening to obtain increased sensitivity. (Mees, "The Theory of the Photographic Process," 1942.) The sensitizers of our invention can be added to the emulsion before the final digestion or after-ripening, or they can be added immediately prior to coating.

30 The quantity of the particular formamidine sulfenic acid (or salt) added to the photographic silver halide emulsions can be varied, depending upon the effect desired, degree of ripening, silver halide content of the emulsion, etc. The amount used will also depend upon at what stage the sensitizer was added during the preparation of the emulsion. We have found that generally from about 0.02 to about 20 mg. of formamidine sulfenic acid per mole of silver halide is quite satisfactory to accomplish the sensitization desired, if added before the final digestion. The N-substituted derivatives can be employed in somewhat larger amounts, and generally as much as 250 to 300 mg. can be added to the emulsions before digestion. On the other hand, somewhat larger amounts are required when the formamidine sulfenic acids or their salts are added to the emulsions immediately prior to coating. Under such conditions, from about 10 to 400 mg. of sensitizer can be added. The most useful or optimum amount of sensitizer to be used can be determined by preparing a series of test strips of the same emulsion, wherein the quantity of sensitizer is varied. It is to be

## 3

understood that the above amounts are given as typical ones, and that we have found in general that sensitization can be realized when the sensitizers are added within the ranges suggested above, although the optimum amount for a given compound might lie outside of the ranges given. It has also been noted that increased sensitization can be obtained, and that larger quantities of sensitizer can be employed, in cases where the final ripening of the silver halide emulsion is carried out for longer periods of time than normal, but at lower ripening temperatures. This observation has been particularly noticeable in the case of formamidine sulfonic acid itself, and less noticeable in other cases.

There appears to be some reaction in the nature of a hydrolysis when the formamidine sulfonic acids of our invention are added to water, or aqueous alkaline solutions. Just what chemistry is involved when these sensitizers are contacted with water is not clear, since the aqueous composition resulting from such addition is a number of compounds difficult to identify. Unsubstituted formamidine sulfonic acid appears to undergo spontaneous reaction with water, whereas certain of the N-substituted derivatives undergo reaction only when the water is warmed or alkali (e.g., sodium hydroxide, sodium carbonate) is added. Thus in certain instances, the sensitizers used in our invention can be characterized as hydrolysates of formamidine sulfonic acids.

The formamidine sulfonic acids useful in practicing our invention can be added to the emulsions to be sensitized either as a solid, or in admixture with water. When added as a solid, the formamidine sulfonic acid combines evidently with the water present in the emulsion to give the desired sensitizing effect. Alternatively, the particular formamidine sulfonic acid can be added to an aqueous alkaline solution, and either allowed to stand or heated slightly to effect solution.

The photographic silver halide emulsions used in practicing our invention are generally of the developing-out type. It is to be understood that the amount of silver halide in the emulsions can be varied, depending upon the particular purpose for which the emulsion is to be employed. Particularly useful results can be obtained when at least one formamidine sulfonic acid is employed in conjunction with gelatino-silver-bromide emulsions, although they can also be advantageously employed in sensitizing other silver halide emulsions, such as gelatino-silver-chloride, -bromide, -chlorobromide, -chlorobromodide, etc., emulsions.

The photographic silver halide emulsions used in practicing our invention can also be optically sensitized by means of the dyes customarily employed in photography, such as cyanine dyes, carbocyanine dyes, dicarbocyanine dyes, merocyanine dyes, holopolar dyes, etc. The sensitizing effect obtained in our invention is not completely independent of the optical or spectral sensitizing dyes commonly used, although no adverse effects have been noted in using emulsions which have been optically sensitized. Also, the formamidine sulfonic acids of our invention can be employed in conjunction with other chemical sensitizers.

The photographic silver halide emulsions employed in practicing our invention can also contain antifoggants or materials known to stabilize the emulsions against loss of speed under adverse keeping conditions, such as those customarily encountered in the tropics. Such antifoggants include, for example, those described in Allen et al. U.S. application Serial No. 586,654, filed May 23, 1956, as well as many of the antifoggant compounds which can be generally classed as polyazaindenes. Such polyazaindenes have been described in U.S. Patents 2,444,605-9; 2,743,181; 2,735,769; etc.

The photographic silver halide emulsions employed in our invention can be used in the preparation of materials, such as multilayer materials, intended for use in color photography, where a number of separate silver halide

## 4

emulsion layers are sensitized for a particular region of the spectrum. Such multilayer color materials generally have a red-sensitive layer coated on a support, followed by a green-sensitive layer, a blue light-absorbing layer, and a blue-sensitive layer, together with one or more interlayers comprising gelatin or some other colloid having various addenda, such as ultraviolet absorbing agents, etc., incorporated therein. These light-sensitive layers can contain color-forming materials of the type customarily employed in color photography, such as coupling compounds containing reactive ketomethylene groups, phenolic groups, or heterocyclic groups, such as pyrazolone. See, for example, U.S. Patent 2,640,776. These color-forming compounds can be incorporated in water-insoluble, low molecular weight, organic, crystalloidal materials having a boiling point above about 175° C., such materials being of the type described in U.S. Patent 2,322,027.

It has been found that the chemical sensitizers of our invention are useful in combination with emulsions which have been sensitized with gold salts, such as those described in Waller and Dodd U.S. Patent 2,399,083, or Damschroder U.S. Patent 2,597,856 or Yutzy and Leermakers U.S. Patent 2,597,915 (e.g., potassium chloraurite, potassium aurithiocyanate, potassium chloroaurate, auric trichloride, 2-aurosulfobenzothiazole methochloride, etc.). Also, emulsions which have been sulfur-sensitized, such as by the procedures shown in Sheppard U.S. Patent 1,574,944 or U.S. Patent 1,623,499 or Sheppard and Brigham U.S. Patent 2,410,689 can be employed in our invention. Such sulfur-sensitized emulsions can additionally contain gold sensitizers of the type mentioned above, or gold compounds intended primarily for stabilization purposes.

35 The following examples will serve to illustrate more fully the manner of practicing our invention:

## Example 1

40 A fine-grain, low-gelatin, positive speed bromide emulsion was prepared and washed by the acid coagulation method described in U.S. Patent 2,614,928. The pH of the emulsion was then adjusted to 6.0 and the emulsion held for 50 minutes at 60° C., both in the absence and presence of formamidine sulfonic acid. Additional gelatin and a coating aid, such as saponin, were then added and the emulsion coated on a suitable support, such as glass, cellulose acetate film, polyvinyl resin film, etc. After drying, the coatings were exposed for 1/25 second positive on an Eastman Type Ib sensitometer and developed for 6 minutes at 70° F. in a developer having 50 the following composition:

|                                | G.   |
|--------------------------------|------|
| N-methyl-p-aminophenol sulfate | 0.3  |
| Hydroquinone                   | 6.0  |
| Sodium sulfite (dry)           | 38.0 |
| 55 Sodium bisulfite            | 1.5  |
| Sodium carbonate monohydrate   | 22.0 |
| Sodium bromide                 | 0.78 |
| Citric acid                    | 0.7  |
| Water to make one liter.       |      |

60 The speed contrast and fog for each of the emulsion coatings was measured, comparison being made between the coating containing no formamidine sulfonic acid, and coating containing formamidine sulfonic acid in the quantities indicated below (the amount being on the basis of per mole of silver halide present). The results follow:

| Coating  | Formamidine sulfonic acid (mg./mole AgX) | 30/E Speed | Gamma | Fog |
|----------|------------------------------------------|------------|-------|-----|
| (a)----- | None                                     | 1.20       | 0.36  | .05 |
| (b)----- | 0.5                                      | 4.10       | 1.28  | .05 |
| (c)----- | 1.5                                      | 5.25       | 1.33  | .05 |

## Example 2

A fine-grain emulsion prepared in exactly the manner shown in Example 1, except that the final digestion was for 1 hour at 40° C., was treated in the presence and absence of formamidine sulfonic acid in the amounts indicated below. Speed, gamma and fog of each of the resulting coatings were measured as in Example 1. The results follow:

| Coating  | Formamidine sulfonic acid (mg./mole AgX) | 30/E Speed | Gamma | Fog |
|----------|------------------------------------------|------------|-------|-----|
| (a)----- | None                                     | 1.90       | 0.46  | .04 |
| (b)----- | 5.0                                      | 4.80       | 1.28  | .05 |
| (c)----- | 10.0                                     | 6.60       | 1.30  | .04 |

## Example 3

A fine-grain photographic emulsion was prepared according to the method described in Example 2, except that the emulsion was then sulfur-sensitized, for example, as described in U.S. Patent 1,574,944. A batch of this emulsion containing no formamidine sulfonic acid sensitizer was then compared with an identical batch containing the sensitizer in the amounts indicated below. Exposure and development was identical to that of Example 1. The results follow:

| Coating  | Formamidine sulfonic acid (mg./mole AgX) | 30/E Speed | Gamma | Fog |
|----------|------------------------------------------|------------|-------|-----|
| (a)----- | None                                     | 22.80      | 3.03  | .05 |
| (b)----- | 5.0                                      | 52.5       | 3.80  | .06 |

Examples 4, 5 and 6 below illustrate the effects obtained when the formamidine sulfonic acids of our invention are added after the final digestion, but before coating.

## Example 4

A high-speed bromiodide emulsion which had been chemically sensitized with sulphur and gold compounds was modified by adding thereto, after the final digestion but before coating, a formamidine sulfonic acid in the amount indicated in the following table. The emulsions were then coated on a conventional support, such as glass or cellulose acetate, and the coatings dried. The coated emulsions were then exposed in an Eastman Type Ib sensitometer for  $\frac{1}{25}$  second and then processed for 5 minutes in a developer having the following composition:

|                                | G.   |
|--------------------------------|------|
| N-methyl-p-aminophenol sulfate | 2.5  |
| Hydroquinone                   | 2.5  |
| Sodium sulfite (dry)           | 30.0 |
| Sodium borate                  | 10.0 |
| Potassium bromide              | 0.5  |
| Water to make one liter.       |      |

The speed, contrast and fog of each of the emulsion coatings was measured, comparison being made between the coating containing no formamidine sulfonic acid and coatings containing a formamidine sulfonic acid in the quantities indicated below (the amount being on the basis of per mole of silver halide present). The speed figure (CR) used in the table is on the basis of 100 (1-log E), where E is the exposure in meter-candle-seconds of daylight quality radiation required to produce a developed density of 0.30 above fog.

| Coating  | Addenda (g./mole AgX)                    | Fresh Tests |       |     |
|----------|------------------------------------------|-------------|-------|-----|
|          |                                          | CR Speed    | Gamma | Fog |
| (a)----- | None                                     | 302         | 1.36  | .12 |
| (b)----- | Formamidine sulfonic acid (.03)          | 315         | 1.34  | .15 |
| (c)----- | N-methyl formamidine sulfonic acid (.03) | 302         | 1.34  | .11 |
| (d)----- | N-methyl formamidine sulfonic acid (.15) | 306         | 1.15  | .11 |

## Example 5

In exactly the manner shown in Example 4 above, and to the same type of emulsions, were added varying amount of formamidine sulfonic acids useful in practicing our invention. Development was as described in Example 4. The following results were obtained:

| Coating  | Addenda                    | Concen-tration (g./mole AgX) | Fresh Tests |       |     |
|----------|----------------------------|------------------------------|-------------|-------|-----|
|          |                            |                              | CR Speed    | Gamma | Fog |
| (a)----- | None                       | None                         | 298         | 1.23  | .11 |
| (b)----- | Formamidine sulfonic acid  | 0.03                         | 301         | 1.14  | .23 |
| (c)----- | N-methyl derivative of (b) | 0.03                         | 302         | 1.24  | .13 |
| (d)----- | do                         | 0.15                         | 311         | 1.19  | .13 |
| (e)----- | do                         | 0.3                          | 314         | 1.14  | .17 |

## Example 6

In exactly the manner illustrated in Example 4 above, an ordinary high-speed bromiodide emulsion was treated with one of the compounds useful in practicing our invention. Instead of adding the compound directly to the emulsion as shown in Examples 4 and 5, the N-ethyl derivative shown in the table below was added to a dilute aqueous alkaline solution and warmed until solution was effected. The alkaline solution was then added to the emulsion immediately prior to coating and thoroughly mixed therewith. Processing was exactly as described in Examples 4 and 5 above. The results obtained were as follows:

| Coating  | Addenda                                                   | Concen-tration (g./mole AgX) | Fresh Tests |       |     |
|----------|-----------------------------------------------------------|------------------------------|-------------|-------|-----|
|          |                                                           |                              | CR Speed    | Gamma | Fog |
| (a)----- | None                                                      |                              | 297         | 1.10  | .10 |
| (b)----- | Alkaline hydrolysate of N-ethyl formamidine sulfonic acid | 0.15                         | 312         | 1.07  | .21 |

In Example 4 above, the pH of the emulsion was adjusted to about 6.3 prior to the addition of the formamidine sulfonic acid, while in Example 5 the pH was adjusted to about 7.1 or 7.2 before adding the sensitizing compound. In Example 6, the pH of the emulsion used was about 6.3 prior to addition of the alkaline hydrolysate.

In Examples 7 and 8 above, the effect of several of the formamidine sulfonic acids useful in practicing our invention is illustrated.

## Example 7

A fine-grain, low-gelatin, positive speed bromiodide emulsion containing no added sulphur or gold sensitizers was prepared as described in Example 1 above. The emulsions were held at the temperatures and times indicated in the following table, both in the absence and presence of a formamidine sulfonic acid. The digested coatings containing sensitizer were then coated on conventional cellulose acetate film and dried. The coatings were then exposed for  $\frac{1}{25}$  second on an Eastman Type Ib sensitometer and developed for 6 minutes at 70° F. in

a developer having the composition shown in Example 1 above. The speed (30/E), gamma and fog for each of the coatings are given in the following table.

| Coating  | Compound                                         | Concen-<br>tration<br>(mg./mole<br>AgX) | Finishing<br>Conditions | 30/E<br>Speed | Gamma | Fog |
|----------|--------------------------------------------------|-----------------------------------------|-------------------------|---------------|-------|-----|
| (a)----- | None                                             | None                                    | None                    | 2.20          | 0.99  | .04 |
| (b)----- | Formamidine sulfonic acid                        | 0.5                                     | 60° at 60 C             | 5.70          | 2.50  | .04 |
| (c)----- | N-methyl derivative of formamidine sulfonic acid | 0.5                                     | do                      | 3.0           | 1.68  | .04 |
| (d)----- | Formamidine sulfonic acid                        | 2.0                                     | do                      | 6.90          | 2.74  | .04 |
| (e)----- | N-methyl derivative of formamidine sulfonic acid | 2.0                                     | do                      | 4.75          | 2.28  | .04 |
| (f)----- | do                                               | 10.0                                    | do                      | 6.30          | 2.72  | .04 |

*Example 8*

A fine-grain, positive speed bromiodide emulsion was prepared and treated exactly as described in Example 7 above. The emulsions containing sensitizer were digested for the times indicated and their properties, after exposure and development, were compared with an untreated emulsion just as described in Example 7. The results obtained were as follows:

| Coating  | Compound                                        | Concen-<br>tration<br>(mg./mole<br>AgX) | Finishing<br>Conditions | 30/E<br>Speed | Gamma | Fog |
|----------|-------------------------------------------------|-----------------------------------------|-------------------------|---------------|-------|-----|
| (a)----- | None                                            | None                                    | None                    | 1.26          | 0.88  | .04 |
| (b)----- | N-ethyl derivative of formamidine sulfonic acid | 10.0                                    | 60° at 60 C             | 4.73          | 2.72  | .04 |
| (c)----- | do                                              | 20.0                                    | do                      | 5.40          | 2.70  | .04 |
| (d)----- | do                                              | 40.0                                    | do                      | 6.60          | 3.16  | .04 |
| (e)----- | do                                              | 100.0                                   | 60° at 40 C             | 3.75          | 2.70  | .04 |
| (f)----- | do                                              | 250.0                                   | do                      | 6.80          | 3.24  | .04 |

The above examples illustrate the effect obtained with our novel sensitizers in acid or alkaline emulsions. When employing these sensitizers in alkaline emulsions, it is to be understood that alkali metal salts thereof may be formed and that these salts exist in ionic form. As indicated above, certain of these sensitizers appear to undergo reaction with the water, and for this reason they have been referred to above and in the following claims as hydrolysates. Accordingly, it is to be understood that use of our sensitizers in photographic emulsions contemplates the use thereof in acid or alkaline emulsions. As indicated above, these photographic emulsions can be sensitized or not by means of optical sensitizing dyes. Such photographic emulsions can be orthochromatic, panchromatic or X-ray emulsions. If used with spectral (optical) sensitizing dyes, the sensitizers of our invention can be added to the emulsion before or after such dyes are added. Suitable dispersing agents for the silver halide emulsions according to our invention comprise gelatin or other colloids, such as collodion, albumen, cellulose organic derivatives, synthetic resins, etc. The sensitizers of our invention can also be used in emulsions adapted for use in color photography, such as emulsions coated in sequence on a single support and being sensitized to particular regions of the spectrum. The emul-

sions may or may not contain couplers or color-forming compounds, which combine with the oxidation products of color developers to produce colored images.

bearing a complementary relationship to the exposing source.

As indicated above, the sensitizers of our invention can be employed in photographic silver halide emulsions containing stabilizers or antifoggants. For example, compounds comprising either the thiazolidine (I) or the tetrahydrothiazine (II) nucleus are useful antifoggants, contrast raisers, or sensitizers in photographic emulsions:



The nucleus is joined in the 3:4 position to a five or six-membered ring which may contain carbon, nitrogen, oxygen, etc., e.g., in which:



$n=1$  or  $2$

$R_3=H$ , alkyl, aryl, e.g. phenyl

$:X=S$  or  $:O$

$-Z=S-$  or  $-SO_2$  or  $SO-$

$R_4$  and  $R_5=H$ , alkyl, phenyl, carboxyl, etc.

The photographic activity of a typical compound, the hydantoin of 4 carboxythiazolidine [ $n=1$ ;  $R_3$ ,  $R_4$ ,  $R_5=H$ ;  $X=O$ ;  $Z=S$  in above structure], is shown in the following table for two different emulsions.

| Emulsion                   | Addendum<br>Concen-<br>tration<br>Per Mole<br>of Silver | Fresh Tests       |                      |                    |                      | Two-Week Incubations<br>at 120° F./50% R.H. |              |                      |
|----------------------------|---------------------------------------------------------|-------------------|----------------------|--------------------|----------------------|---------------------------------------------|--------------|----------------------|
|                            |                                                         | CR<br>Speed       | Gamma                | Maximum<br>Density | Fog                  | CR<br>Speed                                 | Gamma        | Fog                  |
| Slow unsensitized Chloride | G.                                                      | -246<br>-172      | 0.65<br>1.00         | 0.82<br>1.08       | 0.04<br>0.04         |                                             |              |                      |
| Negative type Bromoiodide  | 0.015<br>0.030                                          | 290<br>302<br>291 | 1.18<br>1.12<br>1.02 |                    | 0.11<br>0.11<br>0.09 | 263<br>251                                  | 0.94<br>0.87 | >1.0<br>0.46<br>0.50 |

The hydrolysates used in our invention can be prepared as follows:

5.0 mg. of N-ethylthiourea dioxide were dissolved in 10 cc. H<sub>2</sub>O at room temperature, then 0.2 cc. of a .25 N sodium hydroxide solution were added and the solution heated to 60° C. as rapidly as possible on an electric hot plate and removed as soon as the above temperature had been obtained. The solution was then diluted to 20 cc. and used directly.

What we claim as our invention and desire secured by Letters Patent of the United States is:

1. An unexposed photographic silver halide emulsion sensitized by addition thereto of an aqueous hydrolysate of a compound selected from those represented by the following general formula:



wherein M represents a member selected from the class consisting of a hydrogen atom and an alkali metal atom, and R, R<sub>1</sub> and R<sub>2</sub> each represents a member selected from the class consisting of a hydrogen atom and a hydrocarbon radical, provided that at least one of the members selected from the group consisting of R, R<sub>1</sub> and R<sub>2</sub> represent a hydrocarbon radical, said aqueous hydrolysate having been prepared by heating a compound selected from those represented by said general formula in the presence of water.

2. An unexposed photographic silver halide emulsion sensitized by an aqueous hydrolysate of the N-methyl derivative of formamidine sulfonic acid, said aqueous hydrolysate having been prepared by heating the N-methyl derivative of formamidine sulfonic acid in the presence of water.

5. An unexposed photographic silver halide emulsion sensitized by an aqueous hydrolysate of the N-ethyl derivative of formamidine sulfonic acid, said aqueous hydrolysate having been prepared by heating the N-ethyl derivative of formamidine sulfonic acid in the presence of water.

10. An unexposed photographic silver halide emulsion, gold and sulfur sensitized to its optimum by a gold compound and a sulfur compound, said photographic silver halide emulsion being additionally sensitized by an aqueous hydrolysate of a compound selected from those represented by the following general formula:



wherein M represents a member selected from the class 20 consisting of a hydrogen atom and an alkali metal atom, and R, R<sub>1</sub> and R<sub>2</sub> each represents a member selected from the class consisting of a hydrogen atom and a hydrocarbon radical, provided that at least one of the members selected from the group consisting of R, R<sub>1</sub> and R<sub>2</sub> represents a hydrocarbon radical, said aqueous hydrolysate 25 having been prepared by heating a compound selected from those represented by said general formula in the presence of water.

30 References Cited in the file of this patent

UNITED STATES PATENTS

|              |                    |               |
|--------------|--------------------|---------------|
| 2,262,055    | Sease et al. ----- | Nov. 11, 1941 |
| 2,339,309    | Weber et al. ----- | Jan. 18, 1944 |
| 35 2,376,297 | Weber -----        | May 15, 1945  |